

Dec. 25, 1945.

F. R. HENSEL

2,391,455

SPARK PLUG AND ELECTRODE THEREFOR

Filed June 22, 1943

Fig. 1

NICKEL, IRON  
OR COPPER ALLOY



TUNGSTEN OR  
TUNGSTEN BASE  
METAL COMPOSITION

10

11 PLATINUM  
ALLOY

NICKEL, STEEL  
OR NICKEL  
ON COPPER

13

Fig. 3



TUNGSTEN  
OR TUNGSTEN  
BASE

11

30

PLATINUM  
ALLOY

Fig. 2



1

1

1



BASE  
METAL

PLATINUM  
ALLOY

Fig. 4

INVENTOR.

Franz R. Hensel

BY

Rollin & Carlson

ATTORNEYS

## UNITED STATES PATENT OFFICE

2,391,455

SPARK PLUG AND ELECTRODE  
THEREFORFranz R. Hensel, Indianapolis, Ind., assignor to  
P. R. Mallory & Co., Inc., Indianapolis, Ind., a  
corporation of Delaware

Application June 22, 1943, Serial No. 491,748

4 Claims. (Cl. 123—169)

This invention relates to spark plugs and the electrodes therefor.

An object of the invention is to improve spark plugs and the metal compositions used for the electrodes thereof.

Other objects of the invention will be apparent from the description and claims.

## In the drawing:

Figure 1 shows a portion of a spark plug, partly in section, illustrating the spark plug electrodes;

Figure 2 is an end view of the spark plug;

Figure 3 is a section through a portion of a modified plug; and

Figure 4 is an end view of a further modification.

The invention contemplates a spark plug having a center electrode of tungsten or a tungsten base metal composition and a side or ground electrode formed of platinum base alloy.

Referring to Figures 1 and 2, the center electrode may comprise a cylindrical section 11 of tungsten or tungsten base metal rod welded to the end of a nickel, nickel alloy, iron alloy or copper alloy rod 12 which is embedded in the ceramic insulator 13 of the spark plug. The rod 12 may consist of an upper portion of nickel alloy to be welded to the tungsten and a copper backing to extract the heat. The side electrodes 10 may be formed of platinum alloy wire of rectangular or circular cross section spot-welded to the metal shell 14 of the plug.

Figure 3 shows a modification wherein the side electrode is formed of a short section 30 of platinum alloy wire welded to the end of a supporting wire 31 of base metal such as nickel, steel, or a high heat conductivity metal such as copper sheathed with nickel.

In the modification of Figure 4 the side electrodes comprise bimetallic strips having a layer 40 of platinum alloy facing the center electrode welded to a layer 41 of base metal behind it.

An alloy of platinum and molybdenum containing about 4% molybdenum is the preferred material. This alloy has a hardness of about 104 Rockwell B, and an ultimate tensile strength of 117,000 lbs. per square inch. This material may be used in the form of .030 inch square wire cut into pieces about  $\frac{1}{4}$  inch long which are welded onto opposite sides of the spark plug shell. This construction provides two spark gaps at opposite sides of the center electrode 11. This construction is economical and permits easy adjustment of the spark gap. The platinum-mo-

lybdenum alloy can be readily resistance welded to the steel shell 14.

The range of compositions between 0.5 and 7.5% molybdenum, balance platinum, produces the most satisfactory results. However, molybdenum will alloy with platinum in all proportions up to above 40% molybdenum and forms solid solutions of molybdenum in the platinum throughout this range. Compositions in this permissible range of proportions, but outside the preferred range, may in some cases be used.

Platinum molybdenum alloys, when used for spark plug electrodes have the advantages of withstanding the erosive action of the spark resulting in gap growth. In a number of alloys used at present frequent adjustment of the electrodes is necessary due to such gap growth. For long range flying it becomes necessary to have spark plugs which will not need overhauling for long periods of time. Also in high altitude flying the spark gap must remain properly adjusted since otherwise the sparking voltage increases resulting in misfiring.

Another platinum base alloy suitable for the side electrode is a platinum beryllium alloy containing 0.025 to 5% beryllium, balance platinum. The preferred alloy contains 0.20% beryllium. The beryllium has an extraordinary hardening effect on the platinum, as little as 0.05% beryllium giving a hardness equal to that of the 10% iridium-platinum alloy and 0.25% beryllium giving a hardness equal to a 25% iridium-platinum alloy.

Beryllium also improves the resistance of platinum to heat. Platinum-beryllium alloys undergo a much smaller loss in weight on prolonged heating than does pure platinum.

In a spark plug the electrodes are subjected to severe conditions of electric and chemical erosion. In order for the electrodes to have a long life, it is necessary that the alloys used have a high degree of cohesion. The beryllium imparts a very fine grain structure to the platinum and yields an alloy of high tensile strength. Furthermore the high octane fuels will deposit lead oxide which at the sparking temperatures acts as a catalyst for oxygen promoting erosion by oxidation.

Other platinum alloys which can be used are alloys of platinum with rhenium, columbium or tin. All of these materials reduce the volatility of platinum and increases its strength at high temperatures. In the case of platinum-rhenium alloys suitable percentages of rhenium range from 2 to 8% the preferred range extending from

3 to 6%. Rhenium has a similar effect to molybdenum namely increasing the stiffness and erosion resistance of the platinum alloy.

The resistance of platinum to gaseous attack is increased substantially by additions of 0.025 to 10% columbium. The volatility of platinum and its strength at elevated temperatures are improved by the presence of 0.01 to 5% of tin.

It is further contemplated that platinum-chromium alloys containing up to 15% chromium may be utilized since they impart resistance to erosion and strength at elevated temperatures.

It is also considered to use ferromagnetic platinum base alloys characterized by high coercive forces such as 1500-4000 oersteds. A typical composition consists of 23% cobalt or iron, balance platinum. By using permanently magnetized side electrodes the magnetic field will help to stabilize the arc and thereby give more consistent operation.

Further platinum alloys suitable for the purpose of the present invention are manganese platinum alloys with 1 to 15% manganese; platinum palladium alloys with 2 to 20% palladium.

The addition of other elements to platinum up to 15% is permissible provided the performance is not affected. Such other elements may include iridium, rhodium, ruthenium, osmium, tungsten and tantalum.

The center electrode 11 may be formed of fine grained tungsten or a metal composition containing a high percentage of tungsten.

One metal composition which is suitable is formed of

| A          | Per cent |
|------------|----------|
| Molybdenum | 5        |
| Nickel     | 5        |
| Tungsten   | 90       |

The composition can be formed by mixing the metal powders together, pressing the mixture into a compact and heating the compact to a temperature slightly above the melting point of the nickel. Above this temperature the molybdenum dissolves in the nickel and the tungsten particles are rapidly dissolved by the liquid phase but are reprecipitated on certain nuclei developing large round grains. This process continues until all the originally fine tungsten particles have been converted into fairly uniform grains having a diameter about 100 times those of the original particles. All voids are also eliminated in this process and the resulting product, after cooling, is a strong non-porous body of high cohesive strength.

Other tungsten compositions which can be produced by a similar process and which are suitable are:

| B        | Per cent |
|----------|----------|
| Copper   | 5        |
| Nickel   | 5        |
| Tungsten | 90       |

| C        | Per cent |
|----------|----------|
| Gold     | 4        |
| Nickel   | 6        |
| Tungsten | 90       |

Generally the tungsten content may be between 80 and 98% in compositions of this type.

It is often desirable to decrease the work function of tungsten materials used for spark plug electrodes. For this purpose it is contemplated that small proportions of oxides and silicides of alkaline earth metals may be added to the metal compositions during manufacture. However, the

percentage of such ingredients is preferably kept quite small as they have some tendency to promote erosion. The range between .01 and 3% is preferred. Among the alkaline earth compounds which are suitable are calcium-oxide, barium-oxide, calcium silicide, magnesium silicide, strontium oxide.

Another tungsten base material which is suitable for the center electrode is tungsten containing small proportions of boron, alloyed or combined therewith. Instead of boron it is also contemplated that grades of tungsten may be employed containing traces up to several percent of the borides and nitrides of such metals as are contained in the fourth, fifth and sixth group of the periodic system. As an example a tungsten composition containing .50% of zirconium boride may be used. It is further contemplated to use tungsten composition containing tungsten-zirconium compounds in percentages ranging from .01 to about 4 percent.

For certain applications tungsten-uranium compositions are preferred.

The combination of a platinum base side electrode with a tungsten or tungsten base center electrode affords advantages over prior electrode combinations such as nickel versus nickel, nickel versus tungsten; nickel (cobalt, iron) chromium alloys versus itself or nickel because it provides less gap growth, ease of gap adjustment, more consistent sparking voltage and longer electrode life. When tungsten is used as a center electrode the spark plug construction permits a fairly heavy section usually of a diameter of  $\frac{1}{8}$  inch or longer. By a suitable backing to the tungsten it is possible to withdraw the heat and keep the tungsten cool enough so that it will not oxidize. Tungsten operated under such conditions excels all other metals as regards resistance to chemical attack and spark erosion. If tungsten is used however as a side electrode the conditions are quite different. In side electrodes fairly thin sections are used and proper heat transfer cannot readily be provided. The tungsten therefore overheats, oxidizes and wears away very quickly. Furthermore tungsten is very brittle and does not permit gap adjustment. Tests carried out with various tungsten side electrode constructions resulted in breakage of the side electrodes when adjustment was attempted. The difficulties of tungsten side electrodes were overcome by providing a combination as suggested in the present invention. The side electrodes made in accordance with the teaching of this invention can be operated at elevated temperatures without oxidation. The electrodes may be used in thin sections in order to retain a low cost and flexibility of construction to permit gap adjustment. The materials disclosed for side electrodes have excellent resistance to spark erosion. The electrode combination therefore is superior to all prior constructions.

While specific embodiments of the invention have been described, it is intended to cover the invention broadly within the spirit and scope of the appended claims.

What is claimed is:

1. A spark plug for use in aviation engines comprising a pair of spaced electrodes, one of said electrodes being formed predominantly of platinum and the other of said electrodes being formed predominantly of tungsten.

2. A spark plug for use in aviation engines comprising a pair of spaced electrodes, one of said electrodes being formed of a platinum base alloy

and the other of said electrodes being formed of a material selected from the group consisting of tungsten and tungsten base metal compositions containing at least 80% tungsten.

3. A spark plug for use in aviation engines comprising an insulating body, an electrode terminal extending therethrough and terminating in an exposed electrode tip formed predominantly of tungsten, a metal shell encircling said insulating body and a second electrode tip secured thereto and disposed adjacent said first-mentioned electrode tip, the active sparking surface of said second tip being formed predominantly of platinum.

4. A spark plug electrode combination for use in aviation engines comprising a center electrode 15

formed of a material selected from the group consisting of pure tungsten, tungsten-molybdenum-nickel alloy, tungsten-nickel-gold alloy, tungsten-nickel-copper alloy, tungsten-boron alloy, tungsten alloyed with borides and nitrides of elements taken from the fourth, fifth and sixth groups of the periodic table, tungsten-zirconium alloy and tungsten-uranium alloy and a side electrode formed of a platinum base alloy containing an element selected from the group consisting of molybdenum, beryllium, rhenium, columbium, tin, chromium, cobalt, iron, manganese, palladium, iridium, rhodium, ruthenium, osmium, tungsten, and tantalum.

FRANZ R. HENSEL.